

Jan. 12, 1932.

F. A. APGAR

1,841,271

ART OF REFINING HYDROCARBONS

Filed Feb. 10, 1928

2 Sheets-Sheet 1



Jan. 12, 1932.

F. A. APGAR

1,841,271

ART OF REFINING HYDROCARBONS

Filed Feb. 10, 1928

2 Sheets-Sheet 2



## UNITED STATES PATENT OFFICE

FRANK A. APGAR, OF EAST CHICAGO, INDIANA, ASSIGNOR TO SINCLAIR REFINING COMPANY, OF NEW YORK, N. Y., A CORPORATION OF MAINE

## ART OF REFINING HYDROCARBONS

Application filed February 10, 1928. Serial No. 253,513.

This invention relates to improvements in the manufacture of lubricating oils. More particularly, the invention relates to an improved method of distilling and refining lubricating oils which has several important general advantages and which has several special advantages in special applications.

According to the present invention, an oil containing the desired lubricating oil fraction is heated in a still and vapors of the lubricating oil fraction are driven off, the pressure on these lubricating oil vapors is reduced to a value substantially less than atmospheric pressure, the lubricating oil vapors while under this sub-atmospheric pressure are passed through a body of fuller's earth or some similar adsorptive catalyst, and, after passage through the fuller's earth, the vapors are condensed to form a finished lubricating oil distillate. The pressure in the still where the lubricating oil fraction is initially vaporized may be atmospheric, super-atmospheric or sub-atmospheric. The pressure under which the vapors are passed through the fuller's earth may with advantage approximate 15 to 3 inches of mercury absolute; pressures below about 20 inches of mercury absolute are generally useful in carrying out the invention. The operation is with advantage carried out as a continuous operation. The invention includes improvements in the refining operation proper as well as improvements in the combined distilling and refining operation.

Hitherto, it has been customary to refine lubricating oils by treatment with various chemical refining agents, such as sulphuric acid and caustic alkali solutions. Lubricating oils are viscous and usually relatively dense. Also, they frequently tend to form more or less stable emulsions with water or aqueous solutions of refining agents and with sludges resulting from treatment with such agents. These and other peculiar properties of lubricating oils make such refining operations quite critical. The close control required involves difficulties which are emphasized because of the relatively high value of the oil product under treatment.

This invention avoids the difficulties of these

customary methods. The control required is not critical. Such chemical refining agents are not required. Any possibility of contaminating the lubricating oil product with such chemical refining agents is avoided. Loss of valuable lubricating oil components with refining sludges is avoided. The overall losses of lubricating oil are very small. A finished lubricating oil product may be produced directly in a simplified operation from asphalt base crude stocks. The production of finished lubricating oil products from wax-containing stocks may be much simplified. As applied to wax-containing stocks, the invention has moreover several special advantages.

Lubricating oil distillates from paraffine base or mixed base crude stocks usually contain in solution a quantity of wax. The form in which this wax separates from the oil varies and depends upon a number of factors many of which are not yet fully understood. On chilling, such dissolved wax may separate in a so-called "amorphous" state or it may separate in a crystalline state. Until quite recently this phenomena has been explained by assuming two types of wax, an amorphous wax and a crystalline wax. Recently however there is a growing belief that all wax is crystalline but that in the presence of some protective colloid or crystallization inhibitor it separates in an amorphous state. In any event, wax separating in a crystalline state is handled much more easily than wax separating in an amorphous state and several expedients have been used to promote separation of dissolved wax in a crystalline state.

For convenience of reference, wax present under conditions such that it tends to separate as crystalline wax may be designated "potentially crystalline wax" and wax present under conditions such that it tends to separate as amorphous wax may be designated "potentially amorphous wax."

Hitherto, it has been customary to separate potentially crystalline wax by first chilling the oil and then passing the chilled oil through filter presses to separate the resulting wax crystals, a reasonably simple and inexpensive operation. But the usual filter

processes cannot handle potentially amorphous wax. It has been customary to separate potentially amorphous wax by diluting the oil with a low boiling solvent, chilling the mixture, settling or centrifuging the wax from the mixture, and distilling the low boiling solvent from the mixture. To avoid this more complex and more expensive operation, lubricating oil stocks containing potentially amorphous wax have commonly been subjected to a mild cracking to convert potentially amorphous wax to potentially crystalline to permit separation in the manner first described. This cracking, however, tends to reduce the viscosity of the oil and make its color less desirable, so that the lubricating oils so produced are not usually as valuable as those produced without cracking. This invention provides a particularly advantageous method of converting potentially amorphous wax to potentially crystalline wax permitting ready separation by chilling and filter pressing of the refined oil.

When the pressure on the vapors passing from the vaporizing operation to the refining operation proper is reduced, in carrying out the present invention, the vapors are superheated as a consequence. This feature of the invention has several special advantages. It promotes long life of the adsorptive catalyst used in the refining operation. It renders the adsorptive catalyst more effective for its intended purpose, that is the refining of the lubricating oil product, perhaps because this superheating of the vapors reduces condensation in the catalyst body or adsorption by the catalyst of lubricating oil constituents which might otherwise reduce the life or power of the catalyst. Further, due to this superheating of the vapors, they are passed through the adsorptive catalyst at a temperature higher than that corresponding to their boiling point under the prevailing pressure. In the treatment of lubricating oil stocks containing potentially amorphous wax, this seems to be particularly advantageous in promoting conversion of such wax to potentially crystalline wax. In carrying out this invention, this superheating of the lubricating oil vapors is advantageously effected without any possibility of overheating the vapors by reducing the pressure on the vapors before they are passed through the adsorptive catalyst.

The control required in carrying out the invention is not critical, as noted above. For example, since the boiling temperature of a liquid increases with increase of pressure, the temperature of the vapors driven off in the vaporizing still is fixed by fixing the pressure in that still without requiring further control and the temperature of the vapors passing through the adsorptive catalyst is fixed by fixing the pressure in the vaporizing still and the differential between that pressure and the lower pressure in the refining operation prop-

er. The pressure in the vaporizing still may be substantially atmospheric pressure or may somewhat exceed that value, or if the temperature prevailing at such pressure involve objectionable cracking the vaporizing still may be operated under a pressure sufficiently below atmospheric pressure to avoid such objectionable cracking. The temperatures determined by the pressures described, in the treatment of lubricating oil fractions, are particularly advantageous in the combined operation of the invention as well as in the refining operation proper.

The invention will be further described in connection with the accompanying drawings which illustrate, diagrammatically and conventionally, apparatus adapted for carrying out the invention. The exact form of apparatus illustrated is not essential to the invention, but the apparatus illustrated is advantageous for carrying out the invention and it is used for illustration of the invention for that reason. In the accompanying drawings; Fig. 1 represents, in elevation and partly in section, one form of apparatus adapted for carrying out the invention; and Fig. 2 represents, similarly, another form of apparatus adapted for carrying out the invention.

Referring to Fig. 1, the apparatus illustrated comprises a still 3, a reflux tower 4, a refining tower 5, a condenser 6, a receiver 7, and an exhausting pump 8. The reflux tower 4 is of the type described and illustrated in an application of John E. Bell, filed April 1, 1924, Serial No. 703,338. When the valve 9 is opened, vapors from the still pass upwardly through the tower 4, vapors remaining uncondensed escape through connection 10 to a condenser and receiver and reflux condensate, together with any unvaporized portions of oil introduced into the tower, flows back to the still through connection 11. Connections 12 and 13 are provided for introduction of oil into the upper end of tower 4. Connection 14 is provided for draining the tower, or by closing the valve in connection 11 and opening the valve in connection 14 condensate produced in the tower may be discharged without being returned to the still. Connection 15 is provided for the discharge of residual oil from the still. The still 3 may be a fire heated still or a steam heated still or it may be a fire heated still with provision for the introduction of steam into the charge of oil therein. When the valve 9 is closed and the valve 16 is open, vapors from the still escape through connection 17 to and through the refining tower 5. Vapors escaping from the refining tower 5, through connection 18, are condensed in the condenser 6, the condensate being discharged into receiver 7. The refining tower 5, the condenser 6 and the receiver 7 may be maintained under sub-atmospheric pressure by means of the

pressure reducing valve 16 and the exhausting pump 8. Pump 19 is provided for the discharge of condensate through connection 25 when the receiver 7 is under sub-atmospheric pressure. Any material liquefied in the refining tower 5 is run to a storage tank 20 by means of pump 21, either directly through connection 22 or through cooler 23. The vapors supplied through connection 17 may be passed either upwardly or downwardly through refining tower 5 by means of the branch connections shown between tower 5 and the connections 17 and 18. A charge of an adsorptive catalyst, for example, fuller's earth of 40-60 or 60-80 mesh, is supported upon a foraminous partition 24 adapted to retain the adsorptive catalyst but to permit free passage of vapors through the refining tower 5.

In one way of carrying out the invention in the apparatus illustrated in Fig. 1, a crude petroleum or a topped crude petroleum or other lubricating oil stock is first stripped of constituents lighter than suitable as components of the desired lubricating oil product, vapors of these lighter constituents being separately taken off and condensed, and as the lubricating oil vapors begin to come off they are diverted through the refining tower where the latter are subjected to refining treatment in accordance with the invention under sub-atmospheric pressure. The distillation operation, for example, may be carried out as described in an application of Edward W. Isom, filed May 6, 1924, Serial No. 711,376.

The following example will illustrate this mode of operation: The still 3 is initially charged with from one-third to one-half of the normal operating charge of the lubricating oil stock and, with valve 16 closed and valve 9 open, this charge is heated until the lighter constituents of the initial charge have been vaporized and driven off through connection 10. A low boiling fraction, for example, a part of the condensate product from the vapors escaping through connection 10, may be introduced through connection 12 to control the operation. The further introduction of the lubricating oil stock is then begun through connection 13 while the heating is continued. The rate of introduction of the lubricating oil stock through connection 13 is regulated to control the refluxing operation so that only the lighter constituents of the stock are permitted to escape through connection 10. This control may be supplemented by the regulated introduction of a lower boiling fraction, for example, a part of the condensate produced from the vapors escaping through connection 10, through connection 12. Gasoline, kerosene and gas oil components of the lubricating oil stock are stripped from it in this manner. As the distillation continues, a charge of oil containing

the lubricating oil constituents of the stock but free from lighter constituents accumulates in the still 3. Before the charge of oil in the still 3 becomes excessive, the introduction of oil to tower 4 is stopped, the valve 9 is closed and, the exhausting pump 8 being in operation, the valve 16 is open or partly opened, the opening of the valve 16 being regulated to maintain the desired sub-atmospheric pressure in the refining tower 5. The heating is continued and the lubricating oil constituents of the still charge are vaporized and driven off through connection 17. These lubricating oil vapors are passed through the fuller's earth in the refining tower 5 under sub-atmospheric pressure and the vapors of the refined lubricating oil escaping from the refining tower are condensed in the condenser 6 to form a lubricating oil product discharged through connection 25.

If the lubricating oil stock treated in the manner just described contains wax, the discharged lubricating oil product is chilled and put through filter presses for the separation of such wax. This separation is readily effected because of the conversion of potentially amorphous wax to potentially crystalline wax effected in carrying out the invention. It will be apparent that this mode of operation makes possible the production of finished lubricating oil products from wax-containing stocks without re-running of a diluted stock and without any necessity for subjecting the stock to mild cracking as that operation is commonly carried out in so-called "coke" stills.

Referring to Fig. 2, the apparatus illustrated comprises a still 33, a refining tower 35, a condenser 36, a receiver 37 and an exhausting pump 38. The still 33 may be a fire heated still or a steam heated still, for example, as by steam coil 34, or it may be a fire heated still with provision for the introduction of the steam into the charge of oil therein. This still 33 is advantageously arranged for continuous operation as a single unit or as one unit in a battery of continuously operated stills. In continuous operation, the raw stock including the desired lubricating oil product is supplied to the still through connection 26 and the residual oil from which the lubricating oil fraction has been vaporized is discharged from the still through connection 27. Vapors from the still 33 escape through valve 28 and connection 29 to and through the refining tower 35. Vapors escaping from the refining tower 35, through connection 30, are condensed in the condenser 36, the condensate being discharged into receiver 37. The refining tower 35, the condenser 36 and the receiver 37 may be maintained under sub-atmospheric pressure by means of the pressure reducing valve 28 and the exhausting pump 38. Pump 31 is provided for the discharge of condensate

through connection 32 when the receiver 37 is under sub-atmospheric pressure. Any material liquefied in the refining tower 35 is run to a storage tank 39 by means of pump 40, either directly through connection 41 or through cooler 42. The vapors supplied through connection 29 may be passed either upwardly or downwardly through refining tower 35 by means of the branch connections shown between tower 35 and connections 29 and 30. A charge of an adsorptive catalyst, for example, fuller's earth of 40-60 or 60-80 mesh is supported upon a foraminous partition 43 adapted to retain the adsorptive catalyst but to permit free passage of vapors in the refining tower 35.

In one way of carrying out the invention in the apparatus illustrated in Fig. 2, a lubricating oil stock, such as a residual oil remaining after separation of gasoline, kerosene and gas oil from crude petroleum in the preceding stills of a series through which the oil is passed successively, is continuously supplied through connection 26, the desired lubricating oil fraction is vaporized and driven off continuously in the still 33, the remaining residual oil from which the desired lubricating oil fraction has been vaporized is continuously discharged through connection 27, and the lubricating oil vapors as driven off are passed through the refining tower 35 where they are subjected to refining treatment, in accordance with the invention, under sub-atmospheric pressure.

The following example will illustrate this mode of operation: After the still 33 has been brought to an operating balance in the usual way, the vapors of the desired lubricating oil fraction are driven off through connection 29 and these lubricating oil vapors are passed through the fuller's earth in the refining tower 35 under sub-atmospheric pressure maintained by the operation of the exhausting pump 38 and controlled by regulation of pressure reducing valve 28. The vapors of the lubricating oil escaping from the refining tower 35 are condensed in the condenser 36 to form a lubricating oil product discharged through connection 32. The refining operation proper is, like the distilling operation, carried out continuously.

If the lubricating oil stock treated in the manner just described contains wax, the discharged lubricating oil product is put through filter presses for the separation of such wax. Again this mode of operation makes possible the production of finished lubricating oil products from wax-containing stocks without re-running of a diluted stock and without any necessity of subjecting the oil to mild cracking as that operation is carried out in so-called "coke" stills because of the conversion of potentially amorphous to potentially crystalline wax.

It is common practice, at present, to frac-

tionate crude petroleum or topped crude petroleum by passing the oil continuously through a series of stills, progressively heavier fractions being taken off from each succeeding still of the series. This invention may be employed with particular advantage in conjunction with the operation of these stills of such series from which lubricating oil fractions are taken off without interfering with the operation of the still battery. As applied to such operations, the stills from which lubricating oil fractions are taken off are operated under the normal operating pressures and the pressure on the lubricating oil vapors separated in such stills is reduced after the vapors leave the stills.

It will be understood that the usual measuring instruments, such as thermometers and pressure gauges, for example the pressure gauges 44, 45, 46 and 47, are provided as desired or necessary to facilitate observation and control of the operation. Likewise, the apparatus used is with advantage thermally insulated or lagged to minimize heat loss. In particular, the apparatus including the refining receptacle and the vapor connections between the pressure reducing valve (16 or 28) and the condenser (6 or 36) is advantageously lagged or thermally insulated.

Fuller's earth is a particularly advantageous adsorptive catalyst for use in carrying out the invention. Other adsorptive catalysts useful in carrying out the invention include silica gel and other adsorbent earth and clays.

The invention includes the refining operation proper which has been described comprising the passage of lubricating oil vapors through an adsorptive catalyst such as fuller's earth under pressure substantially less than atmospheric pressure, under pressures below about 20 inches of mercury absolute.

I claim:

1. In the manufacture of lubricating oils, the improvement which comprises vaporizing the lubricating oil from a stock containing the same, then reducing the pressure on the vapors, then passing the vapors through an adsorptive catalyst under a pressure below about 20 inches of mercury absolute, and thereafter condensing the vapors to form the lubricating oil product.

2. In the manufacture of lubricating oils from stocks containing potentially amorphous wax, the improvement which comprises vaporizing the lubricating oil from the raw stock, then reducing the pressure on the lubricating oil vapors, then passing the lubricating oil vapors through an adsorptive catalyst under a pressure below about 20 inches of mercury absolute and thereby converting potentially amorphous wax to potentially crystalline wax, and thereafter condensing the vapors to form the lubricating oil product.

3. In the manufacture of lubricating oils, the improvement which comprises vaporizing the lubricating oil and passing the lubricating oil vapors while super-heated through an adsorptive catalyst under a pressure below about twenty inches of mercury absolute.

5 In testimony whereof, I have subscribed my name.

10

FRANK A. APGAR.

15

20

25

30

35

40

45

50

55

60

65